

Aug. 21, 1934.

S. RUBEN

1,971,053

RESISTANCE DEVICE

Filed Jan. 12, 1933

FIG.1.



FIG.2.



INVENTOR-  
SAMUEL RUBEN

BY *W. Holloman*

ATTORNEY-

## UNITED STATES PATENT OFFICE

1,971,053

## RESISTANCE DEVICE

Samuel Ruben, New Rochelle, N. Y.

Application January 12, 1933, Serial No. 651,278

9 Claims. (Cl. 201—76)

This invention relates to a resistance device, and more particularly it relates to a variable resistance device having a resistance element composed of electronically conductive crystals converted from a material of negligible electrical conductivity. The object of the invention is the provision of a rheostat which is durable, is low in production cost and has a wide range of resistance values.

This invention is an improvement upon that described in my co-pending application filed June 10, 1932, and bearing Serial Number 616,437, particularly in respect to the material used and to the manufacture thereof. In my co-pending application the resistance base is composed of a sintered mass of crystals of cuprous oxide having a surface layer of specified compounds. I have found that if a compound of cadmium and an element of the sulphur group, except oxygen, such as cadmium sulphide or cadmium selenide crystals, with a non-conductive filler and a binder are pressed into a hard mass and heated sufficiently in an oxidizing atmosphere, the surface is converted from a relatively non-conductive material into a good electrical conductor because of the conversion of cadmium sulphide or cadmium selenide into cadmium oxide over the surface of the element. Cadmium telluride also may be so oxidized, but its use is not as satisfactory. By varying the time of heating, and the concentration of the oxidizing atmosphere, resistances of various ranges are obtainable. Cadmium oxide is a good electrical conductor having the desirable characteristic of a negligible temperature resistance coefficient. This is quite different from other electronically conductive crystals which have a high negative temperature resistance coefficient.

The preferred method for making this resistance element is to mix cadmium sulphide or selenide with a suitable binder, such as 2% sodium silicate or lead borate, compress the mixture under high pressure into the desired form and heat the mass until it is completely sintered in a non-oxidizing atmosphere such as nitrogen.

For a variable resistance having an exponential relation of resistances along its length, various portions of the surface of the cadmium sulphide or cadmium selenide elements are exposed to an oxidizing heat which converts the contacting portion into cadmium oxide, the time of exposure, the temperature and the concentration of oxygen determining the ultimate electrical resistance value for each area so treated, the resistance decreasing with the temperature, the concentration and time of application. Termi-

nals with a suitable movable contact member are provided.

For a uniform resistance value along the length, the compressed and sintered cadmium compound element is placed in an oxidizing furnace and by continuous measurement, its resistance value can be fixed at any point, when the element is removed from further exposure. Likewise a definite resistance may be fixed over any section. For high resistances I have found that by the addition of a filler of zircite, a hard mass having much higher resistance values is yielded.

Reference is made to the accompanying drawing in which Fig. 1 represents a plan view of a rheostat and Fig. 2 a section view thereof embodying the invention.

Referring more particularly to the drawing, at 1 is a compressed and sintered arcuate resistance plate composed of cadmium sulphide crystals with a binder and having a surface layer of varying thicknesses of cadmium oxide. The plate rests upon an insulating base 2, attached thereto by terminals 3 and 4. A rotatable conductive arm 5, having a contact electrode 6, is mounted upon shaft 7 and connected in a circuit by conductive plate 8 on shaft 7. At 9 is a knob for rotating arm 5 and nut 10, 11 being a compression spring to insure uniform pressure between the resistance element and contact electrode 6.

What I claim is:

1. A resistance element having a base composed of a compound of cadmium with one of the elements sulphur, selenium and tellurium, and having a surface layer composed of cadmium oxide reduced in situ from the said base compound.

2. A resistance element as in claim 1 in which different sectors of the resistance element surface have different resistance values.

3. A resistance element as in claim 1 in which the cadmium oxide varies in depth along the length thereof.

4. A resistance element having a base composed of cadmium sulphide and having a surface layer composed of cadmium oxide reduced in situ from said cadmium sulphide base.

5. A resistance element having a base composed of cadmium selenide and having a surface layer composed of cadmium oxide reduced in situ from said cadmium selenide base.

6. A resistance element having a base composed of cadmium telluride and having a surface layer composed of cadmium oxide reduced in situ from said cadmium telluride base.

7. A variable resistance device comprising a

35

90

95

100

105

110

- base composed substantially of cadmium sulphide and having a surface layer composed of cadmium oxide reduced in situ from said cadmium sulphide, and a contact member adapted to make selective 5 electrical connection with said cadmium oxide surface along its length.
8. A variable resistance device comprising a base composed substantially of cadmium selenide and having a surface layer composed of cadmium oxide reduced in situ from said cadmium selenide, 10

and a contact member adapted to make selective electrical connection with said cadmium oxide surface along its length.

9. The method of making a resistance element which consists in heating a base compound composed of cadmium and one of the elements sulphur, selenium and tellurium, in an oxidizing atmosphere until said base compound surface is reduced to cadmium oxide. 80

SAMUEL RUBEN. 85

15

90

20

95

25

100

30

105

35

110

40

115

45

120

50

125

55

130

60

135

65

140

70

145

75

150